

Aug. 22, 1950

R. ROSEN

2519,792

ELECTROLYTIC PRODUCTION OF METALLIC URANIUM

Filed April 10, 1942



Raphael Rosen Inventor  
By Ph Young Attorney

## UNITED STATES PATENT OFFICE

2,519,792

## ELECTROLYTIC PRODUCTION OF METALLIC URANIUM

Raphael Rosen, Elizabeth, N. J., assignor, by  
mesne assignments, to the United States of  
America as represented by the United States  
Atomic Energy Commission

Application April 10, 1942, Serial No. 438,356

4 Claims. (Cl. 204—64)

1

The present invention relates to the preparation of heavy metals, such as uranium, tungsten and the like by electrolysis and more specifically to the electrolysis of single fluorides of such metals. The invention will be fully understood from the following description of the drawing.

The drawing is a semi-diagrammatic view in sectional elevation of an electric cell for producing metals and especially uranium.

Referring to the drawing, 1 denotes a vessel made of carbon in which the electrolyte is indicated generally at 2. The carbon vessel is preferably the anode of the cell and the positive pole is shown at 3 connected to the positive wire of any convenient source of direct electric current, which source, however, is not shown.

The carbon anode is adapted to be maintained at a high temperature and is for this reason surrounded by insulation 4 in which is embedded electrical heating elements 5. The whole is then surrounded by a steel shell 6. A pipe 7 is provided connecting the interior of the carbon vessel with the outside atmosphere so that gas produced in the electrolysis may be drawn off, as will be disclosed. This gas may be concentrated and collected during the process, although particular apparatus for this purpose is not shown.

The top of the cell container 1 is covered by a cover plate 8 with a central hole 9, through which the cathode 10 projects into the cell interior and well below the surface of the electrolyte. The cover plate is insulated from the cathode by an annular member 11 which surrounds the hole 9 and is provided with an apron which extends down into the hole. This annular member 11 is made of compressed asbestos or other insulating material and, as will readily be understood, prevents all contact between the cathode 10 and the cover plate 8, especially when the cathode is being withdrawn, for example, by the eye bolt 12. A circular shield 13 is rigidly attached to the metal cathode and extends outwardly at right angles to the axis of the cathode so that when the latter is in the cell as shown, this shield fits tightly over the insulating member 11 and completely closes the hole 9 from the atmosphere and thus prevents the escape of gas therefrom. The negative pole of the electrical source is connected at 14.

While the cell described above is quite satisfactory, it may be constructed otherwise and of other materials; for example, the carbon anode may be replaced by other materials such as a container made of beryllium or silicon, but it must be appreciated that these materials will find their

2

way into the electrolyte and thus into the product in small quantities and consequently depending upon the particular use to which the product is to be applied, a judicious selection of the material of the cathode should be made. Similarly, the anode is preferably of metallic molybdenum, but it may be of tungsten or uranium or even of carbon or other non-reactive materials, which materials, however, are good conductors of electricity. Similarly, the cell is shown as being heated electrically but this, while convenient, is not necessary as it may be heated in a bath of lead or fused solids or may be directly fired with gas or oil. One convenient method for heating 10 the cell is to provide circulating legs; that is to say, tubes from the bottom of the cell bath to an upper portion thereof. These tubes are then heated and the electrolyte flows by thermal circulation from the cell through the tubes and back 15 to the cell again. In this manner the temperature can readily be maintained at the desired point.

In the operation of my process which is conducted in batch the electrolyte, consisting of a 20 mixture of alkali or alkaline earth halides, is placed in the cell container and heated to the fusing point. The preferred electrolyte is a mixture of calcium and sodium chlorides. Ordinarily the eutectic mixture, containing about 51.5 mol percent of calcium chloride is employed and this 25 has a fusing point of about 505° C. Any temperature above this may be used so long as it is not high enough to cause volatilization. However, since the bath composition may change from time 30 to time, it is preferred to use a temperature of about 800° C.; that is to say, just above the fusing points of pure calcium chloride and also 35 above that of sodium chloride.

To this bath uranium tetrafluoride,  $UF_4$ , is 40 added from time to time and is decomposed by the action of the electric current. About six volts is required for the cell. The period over which the cell operates may vary considerably but may 45 be conveniently about 30 minutes, during which time all of the uranium or other heavy metal is plated out of the electrolyte in the form of a dark powder which adheres to the metal cathode.

After the metal has been deposited, the current 50 is shut off and the cathode is withdrawn from the cell and the deposited metal may be readily scraped off by any convenient means and is washed with an acid solution and then with water to remove all traces of the electrolyte.

As stated above, the bath consists preferably 55 of the eutectic mixture of calcium and sodium

chlorides and it may be reused time after time. It will, however, gradually be converted to fluorides due to the action of the elemental fluorine which is released at the anode during the electrolysis. Thus, the fluorine which is released will be contaminated with a small amount of chlorine if chlorides are employed in the bath. If it is desired to recover a high purity fluorine gas, it is preferred to employ fluorides as the bath constituent instead of chlorides. The fluorine may then be compressed and recovered in the ordinary manner.

As a practical illustration of the manner in which the present invention operates, the following may be considered. The cell body is a carbon crucible of, say, 16-inch diameter and 16 inches deep. It is heated electrically and maintained at a temperature of about between 800 and 850° C. The electrolyte consists of the eutectic mixture of 51.5 mol per cent calcium chloride and sodium chloride and to this bath is added 40 pounds of uranium tetrafluoride; that is to say, in ratio of 1 pound thereof to 3 pounds of the electrolyte bath. The current is then turned on, using six volts and about 4,000 amperes for a period of about 30 minutes. At the end of this time the uranium is completely deposited. The current is then shut off and the cathode withdrawn from the cell. Approximately 17 pounds of uranium is recovered from the cathode as a dark powder. An additional quantity of uranium tetrafluoride is then added to the bath, the cathode replaced and the current again turned on so that the cycle is repeated.

After a considerable period of time the melting point of the bath gradually increases due to the substitution of the fluoride for the chloride and it may be discarded and replaced.

The present invention is not to be considered as limited by any theory of operation nor to the particular metal produced or materials of construction set forth, but only by the following claims.

I claim:

1. In the process for producing metallic uranium by electrolyzing a uranium salt in a fused bath consisting essentially of mixed alkali and alkaline earth halides, the improvement in which anhydrous uranium tetra fluoride is the uranium salt, said fluoride being introduced into the fused bath in the ratio of 1 part uranium tetra fluoride to 3 parts of said bath, and maintaining a tem-

perature of between about 800° C. and 850° C. during the electrolysis.

2. In the process for producing metallic uranium by electrolyzing a uranium salt in a fused bath consisting essentially of a mixture of sodium and calcium halides, the improvement in which anhydrous uranium tetra fluoride is the uranium salt, said fluoride being introduced into the fused bath in the ratio of 1 part uranium tetra fluoride to 3 parts of said bath, and maintaining a temperature of between about 800° C. and 850° C. during the electrolysis.

3. In the process for producing metallic uranium by electrolyzing a uranium salt in a fused bath consisting essentially of a mixture of sodium and calcium fluorides, the improvement in which anhydrous uranium tetra fluoride is the uranium salt, said fluoride being introduced into the fused bath in the ratio of 1 part uranium tetra fluoride to 3 parts of said bath, and maintaining a temperature of between about 800° C. and 850° C. during the electrolysis.

4. In the process for producing metallic uranium by electrolyzing a uranium salt in a fused bath consisting essentially of a mixture of sodium and calcium chlorides, the improvement in which anhydrous uranium tetra fluoride is the uranium salt, said fluoride being introduced into the fused bath in the ratio of 1 part uranium tetra fluoride to 3 parts of said bath, and maintaining a temperature of between about 800° C. and 850° C. during the electrolysis.

RAPHAEL ROSEN.

REFERENCES CITED

The following references are of record in the file of this patent:

UNITED STATES PATENTS

| Number    | Name          | Date          |
|-----------|---------------|---------------|
| 1,815,054 | Driggs        | July 21, 1931 |
| 1,821,176 | Driggs et al. | Sept. 1, 1931 |
| 1,835,025 | Driggs et al. | Dec. 8, 1931  |
| 1,842,254 | Driggs        | Jan. 19, 1932 |
| 1,861,625 | Driggs et al. | June 7, 1932  |

OTHER REFERENCES

Industrial and Engineering Chemistry, vol. 22, May 1930, pages 516-519.

Mellor: A Comprehensive Treatise on Inorganic and Theoretical Chemistry, vol. XII, publication 1932, pages 74, 75.